

Oct. 29, 1929.

H. R. WILSON

1,733,570

FLOTATION PROCESS

Filed April 3, 1928



INVENTOR

HARRY R. WILSON,

R. Anthony Loring, ATTORNEY

Patented Oct. 29, 1929

## UNITED STATES PATENT OFFICE

HARRY R. WILSON, OF TOOKE, UTAH

## FLOTATION PROCESS

Application filed April 3, 1928. Serial No. 266,910.

In the concentration of certain ores I have found that economy and an improved yield can be obtained by the use of amyl xanthate. This xanthate differs from the xanthates generally used in flotation processes in that it is made with amyl alcohol instead of ethyl alcohol or propyl alcohol.

I have made up the amyl xanthate of approximately the following percentages.

|                   | Per cent |
|-------------------|----------|
| NaOH              | 19.6     |
| Amyl alcohol      | 43.2     |
| Carbon bisulphide | 37.2     |

15 This agent secures improved flotation results in the treatment of oxidized or partially oxidized lead, silver and copper ores.

A specific example is the treatment of tinitic ores. These are silicious oxidized lead-silver ores from the tinitic district in Utah in which the silver is partly combined with the lead and partly in the form of argento-jarosite (a hydrous sulphate of potassium and iron carrying some silver). From this ore a high recovery can be obtained by adding to the pulp amyl xanthate and sodium sulphide, or amyl xanthate alone; that is, without the sulphide though not excluding other agents hereinafter referred to.

30 The accompanying drawing is a flow sheet illustrating such a process. The ore is ground in the usual manner by the use of crushers, rolls, ball mills, etc. The pulp from the ball mill (or rather from the classifier that follows the ball mill) goes to the first cell of the first section. Here amyl xanthate is added, and a concentrate collected. The tails from the first cell go to the second cell, where more concentrate is collected. Amyl xanthate is also added here if necessary.

40 The tails from the second cell go to the third cell, and the operation is repeated in the fourth and following cells. The number of cells used depends on the amount of lead in the ore, and the ease with which it is floated. The concentrates get successively leaner in lead content in the successive cells, so that when the commercial limit of grade of concentrate is reached, the next following cells are used to

50 collect a middling (which is really a poor

grade of concentrate). This middling is returned to the head of the first cell.

The tails from the first section, still fairly rich in lead, go to the first cell of the second section. Here more amyl xanthate is added together with sodium sulphide. A concentrate is collected and the tails go to the second cell of the second section in the same manner as explained above for the first section. The tails from the second cell go to the following cells from which a middling is collected and returned to the first cell. The concentrates from the first section are combined with those of the second section to form the "final" concentrates. The final tails, nearly depleted of lead and silver, go to waste.

The foregoing process has been practiced on several ores and ore mixtures without the addition of a frother or other agent in the first stage. In other ores there have been added in the first stage pine oil as a frother and sodium silicate to "depress", or deaden the flotability of the gangue materials. In ores where the slime and the gangue float easily, sodium silicate is used in order to get a clean concentrate. The crude amyl xanthate has enough frothing power to give a proper froth without the use of pine oil, but where desired pine oil may be advantageously added in small quantities to give more froth, and the silicate to depress certain portions of the ore.

In the second stage, more amyl xanthate is added together with the sulphide. The latter increases the flotability of the lead. It is not all added at once, but in successive stages; part in the first cell, part in the second, and so on. This is advisable because the addition of the entire requirement of the sulphide in the first cell tends to kill the froth, making the bubbles smaller and glassy, like water bubbles, because they carry no metal burden. The quantity of sodium sulphide added has a decided effect on the recovery of lead. The quantity supplied to each cell should be regulated in accordance with the amount of lead contained in the pulp as it reaches the cell in question.

In the case of one ore, a concentrate was made containing lead, 53.9 per cent; silver 100

15.1 ounces per ton and gold 0.22 ounces per ton. For this ore I have used the following quantities per ton of ore treated, namely, sodium amyl xanthate 1 pound; pine oil 0.2 pounds and sodium sulphide 2 pounds. The recovery was 96.2 per cent of the lead, 90.8 per cent of the silver and 80 per cent of the gold.

On another ore, a concentrate was made containing 45.4 per cent of lead and 22.04 ounces per ton of silver. For each ton of ore treated, I have used 2 pounds of sodium amyl xanthate, 5 pounds of sodium sulphide, 1.5 pounds of sodium silicate and 0.03 pound of pine oil.

The reason for making two concentrates or working the process in two stages, as shown on the flow sheet, is because of the manner in which the silver is carried in the ore; partly with the lead and partly in the form of argento-jarosite.

A high recovery of lead and silver can be obtained with amyl xanthate alone or with amyl xanthate together with sodium sulphide. But when the xanthate is used alone it gives a poorer grade of concentrate and more xanthate is required to get the same recovery as when the sulphide is used in conjunction with it. But if the sulphide is added at the beginning of the operation the silver recovery falls off, indicating that the sulphide depressed or impaired the flotation of the argento-jarosite. Tests on ores containing no argento-jarosite showed the same silver recovery whether the sodium sulphide was added at the start or after the collection of the first concentrate.

By using amyl xanthate alone in the first stage of the flotation process, and with the addition of sodium sulphide in the second stage, the lead and silver recoveries were high and the grade of the concentrate excellent from ores containing argento-jarosite.

I have also used amyl xanthate on a low grade copper-silver ore containing oxidized copper, probably a mixture of silicates and carbonates.

The process may be used with advantage also in connection with straight oxide lead flotation and with other oxidized ores. With some oxidized copper ores lime has to be added to give an alkaline pulp. In general with the copper ores sodium sulphide may be added at the start. The usual sort of flotation operations are practiced, such as grinding, agitation and aeration, together with suitable frothing.

Various other proportions of the flotation agents may be used than those specified above. Fusel oil is a commercial or impure amyl alcohol which is cheaper than and may be used instead of pure amyl alcohol in making up the xanthate. Potassium hydroxide may be used in place of sodium hydroxide, but the latter is preferable because it is cheaper.

Various other modifications of the flotation agents and of the methods of treatment may be made without departing from the invention as defined in the following claims.

What I claim is:

1. In the froth floating of an oxidized lead-silver ore containing silver partly combined with the lead and partly in the form of argento-jarosite, the adding of amyl xanthate alone in a first stage and withdrawing a froth concentrate comparatively high in silver, and the adding of amyl xanthate and a sulphide in a second stage and withdrawing a froth concentrate comparatively high in lead.

2. A method of froth floating lead silver ore of the type described which comprises adding amyl xanthate alone in a first stage, withdrawing a froth concentrate comparatively high in silver, adding amyl xanthate and a sulphide in successive following stages, and withdrawing successive froth concentrates comparatively high in lead.

In witness whereof, I have hereunto signed my name.

HARRY R. WILSON.

90

95

100

105

110

115

120

125

130